

## UNITED STATES PATENT OFFICE

HERMAN JOHAN VAN ROYEN, OF HORDE, GERMANY, ASSIGNOR TO FIRM VEREINIGTE STAHLWERKE AKTIENGESELLSCHAFT, OF DUSSELDORF, GERMANY

## PROCESS FOR THE MANUFACTURE OF IRON AND STEEL

No Drawing. Application filed February 16, 1928, Serial No. 254,899, and in Germany February 21, 1927.

This invention relates to a process for the manufacture of iron and steel and has for its object a novel treatment of iron and steel which renders the same quite free from undesirable characteristics.

5 Articles manufactured from hard or mild steel, which must undergo a cold deformation, also undergo a substantial reduction in toughness or tenacity. Cold deformation consists

10 in working the metal at a temperature which is below the temperature of recrystallization. Recrystallization is that change in structure which is produced in cold worked material by annealing the same below the  $Ac_3$  point.

15 This procedure of cold working may be employed in the manufacture of steam boilers, boiler tubes and the like but with the steels hitherto in use this treatment has as a result a reduction in toughness.

20 It may further be noted that ageing of said cold deformed articles further reduces the toughness and tenacity thereof. This reduction of toughness may be observed by means of the impact test on a notched bar.

25 Metallurgists have long been striving to obtain a material which does not have the aforementioned undesirable and unfavorable properties. Up to the present time, however, they have not been able to produce an article

30 which has been subjected to cold deformation, in which the brittleness produced thereby has been confined to tolerable limits and in which the increase of brittleness caused by ageing has been confined to a minimum.

35 Exhaustive investigations made by the inventor, for instance with boiler plates and material for seamless tubes have shown that in this connection it is less a question of the composition and metallurgical purity than a

40 question of the working of the material.

According to the invention a mild or hard steel which is not adversely affected by cold deformation and which resists the increase of brittleness caused by ageing, may be obtained.

45 These results are obtained by virtue of the fact that the working process consists in a deformation operation, rolling, forging or pressing, which is continued to the greatest extent possible at a temperature which is below the  $Ar_1$  point. This deformation takes

place preferably immediately below said  $Ar_1$  point since in the range disposable at these temperatures the material may be deformed to the greatest extent. The next step consists in a normalizing annealing operation carried out at a temperature somewhat above the  $Ac_3$  point. The last operation is cooling in the air.

55 What I claim is:

A process for the manufacture of mild or hard steel insensible against cold deformation and ageing characterized by the fact that the material in the course of its working is deformed as extensively as possible at temperatures lying below its  $A_1$ -transformation-point, the deforming process beginning immediately below the  $Ar_1$ -point and being finished as quickly as possible, after which operation the material is subjected to a normalizing annealing treatment.

60 HERMAN JOHAN VAN ROYEN.

70

75

80

85

90

95

100